

## UNITED STATES PATENT OFFICE

2,044,726

## MANUFACTURE OF LUBRICATING OIL

Francis X. Govers, Vincennes, Ind., assignor to  
 Indian Refining Company, Lawrenceville, Ill.,  
 a corporation of Maine

No Drawing. Application December 24, 1934,  
 Serial No. 758,941

8 Claims. (Cl. 196—17)

This invention relates to the manufacture of lubricating oil from hydrocarbon oils, and more particularly to the manufacture of high viscosity index, low pour test lubricating oil from, wax-  
 5 bearing mineral oils.

In its broadest aspect, the invention contemplates an improved process of treating hydrocarbon oils, particularly paraffin-bearing lubricating fractions of petroleum with solvents to selectively produce therefrom low pour test lubricating oils characterized by having a desired viscosity temperature relationship and improved lubricating qualities. The invention contemplates a process of manufacturing lubricating  
 10 oils having a low pour and cloud test, low sulphur content, low Conradson carbon content, a relatively high viscosity index and free from bodies of little or no lubricating value.

The present application is a continuation-in-  
 20 part of my copending application Serial No. 601,888 filed March 29, 1932 for the Manufacture of lubricating oil.

My above mentioned copending application relates to a process of solvent refining mineral lubricating oil with liquid sulphur dioxide in the presence of a modifying solvent comprising benzol or one of its homologs, or a derivative thereof, such as monochlor-benzol. The present application relates to a process of solvent refining  
 25 mineral lubricating oil with liquid sulphur dioxide in the presence of a modifying solvent comprising a dichlorinated aromatic hydrocarbon such as dichlor-benzene.

Low pour test in a lubricating oil denotes an  
 30 oil, as used in internal combustion engines, possessing the characteristics of easy starting in cold weather and readiness of flow sufficient to respond to methods of circulation so as to immediately reach all parts necessary to be lubricated.

The presence of sulphur or sulphur-containing bodies in lubricating oil is objectionable on account of the corrosive effect of sulphur upon bearing surfaces and other metal portions of the engine. Efforts to reduce the sulphur content of  
 40 lubricating fractions to a desirable degree by methods ordinarily employed have resulted in an over-refined oil with impaired lubricating value.

Lubricating oil having a low Conradson carbon content is desirable since such oil has little  
 45 tendency to carbonize in the motor, and such carbon as may be deposited is of a flocculent nature, having little or no tendency to adhere to the piston head or cylinder walls. High Conradson carbon content is characteristic, for example,  
 50 of residual oils, or oils not redistilled under low

absolute pressure, and is characteristic of oils having desired high viscosity index, as ordinarily produced heretofore.

The viscosity index of a given oil is readily determined by resorting to the method of Dean 5 and Davis, published on pages 618-619 of the 1929 issue of Chemical and Metallurgical Engineering. Lubricating oils of high viscosity index are characterized by having a relatively narrow increase in viscosity with respect to temperature. Such 10 oils have the property of possessing the desired viscosity at elevated temperature with no great loss of mobility at very low temperature.

Lubricating oils, as ordinarily made from naphthenic-base crudes, have a low pour and cloud 15 test, low Conradson carbon content, but have a low viscosity index and fairly high sulphur content. On the other hand, lubricating oils, as ordinarily made from paraffin-base crudes of the Pennsylvania type, have a high pour and cloud 20 test, high Conradson carbon content and a fairly high sulphur content, depending on the particular crude source. Oils derived from mixed base crudes may fall somewhere between these limits although usually high in sulphur content. Oils 25 of the Pennsylvania type, as well as those derived from mixed base crude sources, are difficult to refine without undue loss and impairment of their lubricative value. In any case, it is difficult, by methods now employed, to reduce the sulphur 30 content of lubricating oil fractions to the desired point, regardless of their crude source.

The generally accepted method, as used in the art of refining petroleum lubricants for the removal of sulphur as well as other undesired 35 constituents, is by the use of sulphuric acid. Much stress has recently been put on the danger of over-refining due to the use of this method of refining with its consequent impairment of lubricating value due to over-refinement. Sulphur dioxide has been proposed as a substitute in the refining art but the use of this solvent by itself in refining in viscous fractions, particularly of the paraffin type, has not been successful 40 from the standpoint of producing a product having the desired high viscosity index, low pour test and other characteristics.

I have discovered that by the use of the methods herein disclosed lubricating oils of any desired viscosity index and scale of purification, 50 coupled with low pour test and low cloud test, can be made from mixed-base or paraffin-base crudes, and the oils so produced are characterized further by low Conradson carbon and low sulphur content. The obtaining of oils having 55

these desired qualities does not depend on methods involving redistillation or acid treatment.

More specifically the invention comprises mixing with a wax-bearing fraction of a mineral oil a solvent mixture comprising two or more solvent liquids of differing solvent properties which, in certain ratios of one solvent liquid to other solvent liquids, has substantially complete solvent action on the oil at temperatures of around 10 100-125° F., and at temperatures of around 0° F. substantially complete solvent action on the liquid hydrocarbons therein but substantially no solvent action on the solid hydrocarbons therein, and of such a nature that upon cooling a solution 15 of the mineral oil fraction in such solvent mixture to 0° F. and removing the solid hydrocarbons so precipitated and the solvent liquid the resulting oil has a cold test of substantially 0° F. or below but which solvent mixture in certain other ratios 20 of one solvent liquid to the other solvent liquids has, at temperatures of 32° F. and below, a selective solubility as between differing viscosity index constituents of the liquid hydrocarbon content.

25 The mixture is then chilled to form a precipitate of solid or semi-solid material comprising suspended wax or solid hydrocarbons which are insoluble in, and immiscible with, the solvent mixture. The mother liquor is separated from the cold mixture advantageously by filtration. The 30 separated mass of solid hydrocarbons is then washed free of mother liquor containing dissolved oil by additional quantities of chilled solvent liquid of approximately the same composition as 35 used in the original mix.

A certain portion of the filtrate from this washing operation may be added to the original filtrate, the amount of liquid so added depending on the 40 amount of dissolved oil contained therein. To the original filtrate or mixture of original filtrate and first wash liquor is then added an additional amount of one of the component solvents of the solvent liquid mixture to alter the percentage composition of the components of the solvent mixture in an amount sufficient to affect the solvent 45 capacity of the solvent mixture and cause a separation between soluble and insoluble constituents of the hydrocarbons. This mixture is chilled to effect a sharp and rapid separation into two layers, the upper layer containing oils characterized by relatively high viscosity index, and the lower layer containing oils characterized by relatively 50 low viscosity index. The amount and character of the separation is influenced by the amount of alteration in the percentage composition of the components comprising the solvent liquid mixture.

I have found that a suitable solvent liquid mixture comprises a mixture of liquid sulphur dioxide and dichlor-benzene, and in particular a mixture composed of liquid sulphur dioxide and either ortho or meta dichlor-benzene. A solvent composed of sulphur dioxide and a mixture comprising the isomers of dichlor-benzene may be employed. Para dichlor-benzene which has a relatively high melting point may form a constituent part of the solvent mixture when used in solvent mixtures where it forms a small part of the 65 mixture.

The selective solvent action of a mixture of the solvents upon the various constituents of a hydrocarbon oil fraction is readily altered by varying the proportion of the solvent components of 70 the mixture.

As an example in carrying out the above invention:

200 gallons of untreated vacuum distilled wax distillate having a viscosity of 70 Saybolt Universal seconds at 210° F. with a pour test of 80° F. and a sulphur content of about .4% derived from a semi-paraffin base crude, is mixed with 5 600 gallons of a solvent liquid comprising 30% sulphur dioxide and 70% ortho dichlor-benzene, the mixture is chilled to -15° F. to precipitate the 10 10 wax-like or solid hydrocarbons and introduced to filtering means described in my copending application, Serial No. 585,844, for "Method of and apparatus for filtration", filed January 11, 1932, wherein the solid hydrocarbons are separated from 15 the liquid to produce a filter cake.

A wash solvent liquid comprising 30% sulphur dioxide and 70% ortho dichlor-benzene and chilled to -15° F. is introduced to the press to wash out of the filter cake the adhering mother 20 liquor. The first portion of the filtrate resulting from this washing, which will contain a substantial quantity of dissolved oil may be mixed with the original filtrate, while the remaining portion may be used to mix with fresh untreated 25 wax distillate to be treated in the same manner as the original material as above described.

The slurry remaining in the filter press is then removed and the bulk of the admixed solvent 30 filtered off advantageously by filtering this slurry in a filter means such, for example, as described in my U. S. Patent No. 1,920,126, for "Filtration", issued July 26, 1933. The solvent retained in the resulting filter cake is evaporated 35 from the wax and the wax contacted with clay or finished up in the usual manner.

The wax in the above example will amount to approximately seven and one-half per cent of the original wax distillate and after removal of the solvent by evaporation, steaming in the presence 40 of clay and contact filtering, the wax will be white and have a melting point, without sweating, of about 136° F.

To the mixture of original filtrate and initial portion of wash liquor is added liquid sulphur dioxide chilled to a temperature of -10° F. This additional sulphur dioxide should be sufficient in amount to bring the ratio of sulphur dioxide to ortho dichlor-benzene up to about equal volumes of each.

The mixture is well stirred and allowed to settle and stratify. The top layer will comprise low gravity, relatively high viscosity index oils, while the lower layer comprises high gravity, low viscosity index oils. The oil in the top layer after removal of the solvent will have a gravity of approximately 27.5 A. P. I., a viscosity of 66 Saybolt Universal seconds at 210° F. and a viscosity index of approximately 87. The oil in the bottom layer, after removal of the solvent, will have a gravity of approximately 13 A. P. I., a viscosity of approximately 118 Saybolt Universal seconds at 210° F. and a viscosity index below -30.

The fraction of relatively high viscosity oil may be contacted with clay and filtered, and is then ready for use as a so-called wide cut, or it may be fractionated by vacuum distillation to produce cuts of narrower distillation range.

On the other hand, this relatively high viscosity material may be still further improved or refined by dissolving in ortho dichlor-benzene, cooling the mixture to 0° F. and adding chilled liquid sulphur dioxide in about the same proportion as the dichlor-benzene. The mixture is well stirred, 70 75

chilled to  $-10^{\circ}$  F. and allowed to settle. The oil in the top layer, after removal of the solvent, contacting and steaming in the presence of clay and contact filtering, will have the following approximate characteristics: Gravity 30.6, viscosity of 64 Saybolt Universal seconds at  $210^{\circ}$  F., viscosity index 95, Conradson carbon .015, and sulphur .1, with a pour test of  $-5^{\circ}$  F.

As an additional example in carrying out the above invention:

Untreated vacuum distilled wax distillate, similar to that used in the preceding example, is also similarly mixed with sulphur dioxide and ortho dichlor-benzene in the proportion of about 200 gallons of oil to 600 gallons of solvent mixture, and chilled to  $-15^{\circ}$  F. to precipitate the wax-like or solid hydrocarbons. The mixture is filtered and the resulting filter cake washed with the same fresh solvent in the same manner, the initial portion of the wash filtrate being mixed with the original filtrate.

To this mixture of original filtrate and wash liquor is added chilled sulphur dioxide sufficient to give a solvent mixture of 60% sulphur dioxide and 40% dichlor-benzene. The mixture is stirred well, chilled to  $-10^{\circ}$  F. and allowed to settle and stratify.

The separated bottom layer is drawn off, the solvent evaporated and the oil recovered. There will be recovered an oil having a gravity of approximately 12.4 A. P. I. and a viscosity index of approximately -32.

The separated top layer is mixed with a chilled mixture of ortho dichlor-benzene and sulphur dioxide comprising about 40% sulphur dioxide and 60% dichlor-benzene, well stirred, chilled to  $-10^{\circ}$  F. and allowed to separate. The bottom layer is drawn off, the solvent evaporated and the contained oil contacted at  $500^{\circ}$  F. with 20 pounds of clay to the barrel. This contacting may be carried out in the presence of steam. The oil and clay mixture is cooled to  $350^{\circ}$  F. and filtered. The filtered oil will amount to about 73 gallons and have the following approximate characteristics: Gravity 27.5 A. P. I., viscosity 67 Saybolt Universal seconds at  $210^{\circ}$  F., viscosity index 79½, with a pour test of  $-10^{\circ}$  F.

The solvent is evaporated from the separated top layer and the contained oil contacted at  $500^{\circ}$  F. with 20 pounds of clay to the barrel while steaming. The oil and clay mixture is cooled to  $350^{\circ}$  F. and filtered. The filtered oil will have the following approximate characteristics: Gravity 31.1 A. P. I., viscosity 63 Saybolt Universal seconds at  $210^{\circ}$  F., viscosity index 102, pour test  $-5^{\circ}$  F., Conradson carbon .012, sulphur .09.

The solvent can be recovered from the refined oil by distillation or other means. The sulphur dioxide component may be readily removed by flash distillation while the dichlor-benzene may be removed by distillation under low absolute pressure. It is contemplated also that instead of removing the high boiling solvent liquid from the oil by distillation it may be removed by washing with a suitable solvent liquid adapted to dissolve the solvent and any retained extract phase material remaining in the refined oil. After removal of the wash solvent and dissolved material, the remaining refined oil can then be finished up by contacting with a solid adsorbent material in the presence of steam and at elevated temperature, in accordance with the customary clay contacting type of treatment.

The invention is not limited to the production

of final products having the particular characteristics of those described above. Products of differing characteristics, as desired, may be prepared by varying the proportions of the solvent liquids and also the temperatures at which the treating steps are carried out.

Furthermore, the invention is not limited to the treatment of wax distillate such as given in the examples herein but is adapted to the treatment of other paraffin-containing fractions, precipitates or materials somewhat similar in nature derived in various ways from mineral oils.

Thus my invention is applicable to the treatment of hydrogenation products resulting from the hydrogenation of carbonaceous materials, or mineral oils including liquid or solid hydrocarbon fractions derived from mineral oils. Hydrogenation products may contain substantial quantities of waxy or paraffin material as well as other constituents of relatively low lubricating value. By treating such products in accordance with my invention, final products of desired characteristics can be obtained.

The invention is not restricted to any particular operating conditions such as that of temperature, or the composition of the solvent mixtures employed since these conditions may advantageously be varied, depending upon the nature of the fraction undergoing treatment as well as upon the particular characteristics desired in the final product.

It is also contemplated, in many instances, that it may be of advantage to carry on the filtration step in the presence of a comminuted solid filter-aid material. Such material may be admixed with the chilled mixture of oil and solvent liquid prior to introduction to the filtering means.

While in the foregoing examples the oil is mixed with a mixture of sulphur dioxide and ortho dichlor-benzene, it is contemplated that the wax bearing oil may first be dissolved in the ortho dichlor-benzene alone and then the cold liquid sulphur dioxide added to the mixture.

Obviously many modifications and variations of the invention, as hereinbefore set forth, may be made without departing from the spirit and scope thereof, and therefore only such limitations should be imposed as are indicated in the appended claims.

I claim:

1. The method of dewaxing wax-bearing mineral lubricating oil for the production of oil having a pour test of  $0^{\circ}$  F. and below, which comprises mixing the wax-bearing oil with a solvent mixture comprising liquid sulphur dioxide and dichlor-benzene containing less than 50% sulphur dioxide in proportions such that at temperatures of  $0^{\circ}$  F. and below the mixture has substantially complete solvent action on the liquid hydrocarbon constituents and substantially no solvent action on the solid hydrocarbon constituents of the oil, chilling the mixture to a temperature of  $0^{\circ}$  F. and below to precipitate the solid hydrocarbon constituents and separating the thus precipitated solid hydrocarbon constituents from the cold mixture to thereby produce oil which, after removal of the solvent, has a pour test of  $0^{\circ}$  F. and below.

2. The method of dewaxing wax-bearing mineral lubricating oil for the production of oil having a pour test of  $0^{\circ}$  F. and below, which comprises mixing about one part of wax-bearing oil with three parts of a solvent mixture comprising around 30% sulphur dioxide and the remainder ortho dichlor-benzene in proportions such that

- at temperatures of 0° F. and below the mixture has substantially complete solvent action on the liquid hydrocarbon constituents and substantially no solvent action on the solid hydrocarbon constituents of the oil, chilling the mixture to a temperature of 0° F. and below to precipitate the solid hydrocarbon constituents and separating the thus precipitated solid hydrocarbon constituents from the cold mixture to thereby produce oil which, after removal of the solvent, has a pour test of 0° F. and below.
3. In the manufacture of lubricating oils of desired high viscosity index from mineral oil containing constituents of differing viscosity indices,
- 5 15 the method comprising extracting the oil with a mixture of sulphur dioxide and dichlor-benzene containing up to about 50% dichlor-benzene, forming an extract phase comprising low viscosity index constituents of the oil dissolved in the
- 20 solvent and a raffinate phase comprising relatively high viscosity index constituents of the oil, and separating the two phases.
4. In the manufacture of lubricating oils of desired high viscosity index from mineral oil containing constituents of differing viscosity indices,
- 25 30 the method comprising extracting the oil with a solvent mixture comprising liquid sulphur dioxide and ortho dichlor-benzene, the dichlor-benzene comprising up to about 50% by volume of the solvent mixture, forming an extract phase comprising low viscosity index constituents of the oil dissolved in the solvent and a raffinate phase comprising relatively high viscosity index constituents of the oil, and separating the two phases.
- 35 5. In the process of manufacturing high viscosity index lubricating oil having low pour test from wax-bearing mineral oil, the method which comprises mixing with the oil a solvent liquid mixture composed of liquid sulphur dioxide and dichlor-benzene containing less than about 50% sulphur dioxide in proportions such that at temperatures of 0° F. and below the solvent mixture has substantially complete solvent action on the liquid hydrocarbon constituents and substantially no solvent action on the solid hydrocarbon constituents of the oil, chilling the mixture to a temperature of 0° F. and below to precipitate the solid hydrocarbon, removing the solid hydrocarbons thus precipitated, increasing the proportion of liquid sulphur dioxide to dichlor-benzene in the dewaxed mixture, separating the resulting mixture into a solvent phase containing low viscosity index constituents of the oil dissolved in the solvent, and an oil phase comprising relatively high viscosity index constituents of the oil, and separating the two phases.
- 50 55 6. In the process of separating from wax-bearing mineral lubricating oil a low pour test frac-

tion having a viscosity index of around 100 and above, the method which comprises dewaxing the oil with a solvent mixture comprising liquid sulphur dioxide and dichlor-benzene and containing less than about 50% sulphur dioxide, extracting the dewaxed mixture in the presence of a mixture of sulphur dioxide and dichlor-benzene containing up to about 50% dichlor-benzene having selective action as between naphthenic and paraffinic hydrocarbons and having as a component 10 part of such solvent mixture the solvent liquid retained in the dewaxed mixture, separating from the mixture a raffinate phase comprising paraffinic oil and some solvent, subjecting the separated raffinate phase to further extraction 15 in the presence of sulphur dioxide and dichlor-benzene and separating therefrom a fraction comprising low pour test oil of desired high viscosity index.

7. In the process of separating from wax-bearing mineral lubricating oil a fraction of low pour test having a viscosity index of around 100 and above, which comprises mixing the oil with a mixture of liquid sulphur dioxide and ortho-dichlor-benzene containing less than 50% sulphur dioxide and in proportions such that the mixture 20 has selective action as between wax and oil at temperatures of the order of 0° F. and below, chilling the mixture to separate the wax, removing the wax from the cold mixture, adding further cold liquid sulphur dioxide to the chilled dewaxed mixture, separating therefrom a raffinate phase comprising paraffinic oil and some solvent mixture, subjecting the separated raffinate phase to further extraction in the presence of liquid sulphur dioxide and dichlor-benzene in proportions such that low pour test paraffinic oil of desired 25 high viscosity index is separated therefrom, and removing the solvent from the thus separated oil.

8. In the process of separating from dewaxed mineral lubricating oil a fraction having a viscosity index of around 100 and above, the method which comprises mixing the oil with a mixture of liquid sulphur dioxide and dichlor-benzene containing in excess of 50% sulphur dioxide 40 and in proportions such that the solvent mixture has selective action as between naphthenic and paraffinic hydrocarbon constituents of the oil, separating from the mixture a raffinate phase comprising paraffinic oil and some solvent, subjecting the separated raffinate phase to further extraction with a mixture of sulphur dioxide and dichlor-benzene containing less than 50% sulphur dioxide and in proportions such that oil of desired high viscosity index is separated therefrom.

FRANCIS X. GOVERS.